

3,188,790

## NYLON FIBER BLENDS

Harold H. Hebel, Seaford, Del., assignor to E. I. du Pont de Nemours and Company, Wilmington, Del., a corporation of Delaware  
No Drawing. Filed June 12, 1963, Ser. No. 287,195  
9 Claims. (Cl. 57—140)

This invention relates to new textile products, and is more particularly concerned with a blend of synthetic staple fibers and with its use for blending with and reinforcing natural fibers. This application is a continuation-in-part of my copending application Serial No. 152,314, filed November 14, 1961, as a division of my application Serial No. 668,718, which was filed June 28, 1957, and issued as U.S. Patent No. 3,044,250 on July 17, 1962.

The preparation of uncrimped staple fiber, of synthetic linear condensation polymer, suitable for blending with natural fibers such as cotton to impart both improved abrasion resistance and increased tensile strength, is fully described in my U.S. Patent No. 3,044,250. This patent discloses that, to obtain yarns of good strength from blends of nylon or polyester staple and cotton, it is necessary for the staple fibers to possess high load-bearing capacities at low elongations in the general range of the break elongation of cotton (about 7%). Suitable fibers are prepared from undrawn nylon by a special drawing and heat-treating process in which the fibers are drawn at substantially the maximum operable draw ratio while simultaneously being heated, the product of the temperature of heating in degrees centigrade and the time of heating in seconds being at least about 200 and preferably from about 1000 to 6000. The resulting fibers are characterized by being highly oriented and highly crystalline. The fibers are not crimped because the heat required in conventional crimping processes would produce an amount of relaxation in these nylon fibers which results in too much loss of load-bearing capacity at low elongations.

In the preparation of yarns from blends of different types of fibers, one has a choice of several points in the process at which the different fibers may be brought together. For example, the fibers may be mixed before they are supplied to the picker hopper, they may be processed separately through breaker laps and the blend made on the finisher picker, or the different fibers may be processed separately into sliver and combined on the draw frame. The most economical operation, with the formation of the least amount of mixed waste fiber, involves blending at the draw frame. However, when using highly oriented and crystalline nylon staple fibers, blending at the draw frame has required that uncrimped staple fiber be processed through the picking and carding operations. Unfortunately, it has been found that the carding of this uncrimped nylon staple is accompanied by excessive loading of the main cylinder of the card, especially when metallic clothing is used, and by poor web and lap cohesion, with the result that this potentially economical method of preparing a blended nylon and cotton yarn has not been practicable.

The present invention provides a method of overcoming this problem in preparing nylon/cotton blends. The invention is also applicable to preparing blends of other fibers, such as polyethylene terephthalate staple fiber and cotton. However, since crimped fibers of polyethylene terephthalate can readily be prepared to have load-bearing capacities higher than cotton at low elongations, there will normally be no reason to use any uncrimped polyester staple fibers. Therefore, the disclosure will be concerned primarily with the special problem of preparing nylon blends.

It is an object of this invention to provide a nylon

staple fiber product of improved cardability, suitable for forming nylon/cotton blend yarns of high strength and abrasion resistance. Another object is the use of the product to provide improved processability on cotton system equipment for reinforcing natural fibers. A further object is to make possible more economical production of high strength blended staple yarns. Further objects will appear as the description of the invention proceeds.

It has now been discovered that the picking and carding of uncrimped nylon staple fibers is greatly facilitated by the addition of relatively small quantities of crimped nylon staple fibers. Therefore, the objects of this invention are obtained by a combination of crimped and uncrimped nylon staple fiber comprising 50 to 90% of an uncrimped nylon staple fiber characterized by having both a high degree of crystallinity and a high degree of crystalline orientation such that it has a time-stable load-bearing capacity at least equal to that of cotton fibers at the break elongation characteristic of cotton fibers, and 50-10% of a crimped nylon staple having a crimp index of at least 8%.

Surprisingly, the nylon staple of this invention achieves improved processability in the picking and carding operations while at the same time affording superior reinforcing properties for natural fibers, such as cotton, in blended staple yarns.

The term "nylon" as used herein refers to high molecular weight fiber-forming polycarbonamides, e.g., polyhexamethylene adipamide ("66" nylon) and polycaproamide ("6" nylon).

The uncrimped high load-bearing nylon fiber component of the staple of this invention is that described in my U.S. Patent No. 3,044,250, and may be prepared by methods described therein. The fiber is characterized by a density higher than about 1.139 gm./cc. and a birefringence above about 0.0590. The fiber is further characterized by a load-bearing capacity at an elongation of 7% (hereinafter designated  $T_7$ ) greater than 2.1 grams per denier, measured after 9 days' slack aging. The nylon staple is further characterized by a boil-off shrinkage (shrinkage determined by boiling a previously measured skein in water for 60 minutes) of less than about 6%. The term "uncrimped fiber," as used herein, means a fiber having a crimp index of substantially zero.

Crimp index is determined on individual filaments by (a) straightening a fiber to remove crimp without substantial elongation of the fiber, (b) measuring the straightened length, (c) allowing the fiber to retract freely and again measuring; the crimp index is calculated as follows:

$$\frac{\text{Length (a)} - \text{length (c)}}{\text{Length (a)}} \times 100\% = \text{crimp index}$$

The crimped nylon fiber component of the staple of this invention is characterized chiefly by its crimp index, which is preferably in the range from 15% to 30%. Fiber which has a crimp index less than about 8% does not give the improved processability characteristic of the staple of this invention. While fiber having a crimp index greater than 30% can be used to provide improved processability, it is not as desirable for this purpose, although its use may sometimes be preferred for other reasons.

The crimp of the crimped fiber can be of any of the conventional types, of which the most common is the flat zig-zag crimp produced by a stuffer box crimper as disclosed in Hitt U.S. Patent No. 2,311,174 and Spence et al. U.S. Patent No. 2,917,784. Any of the types of crimp covered in Miles U.S. Patent No. 2,197,896 are suitable, among which may be mentioned the regular crimp produced by gear crimping and the helical crimp produced by

twisting and heat setting. The production of helical crimp with false twisting apparatus is disclosed in Breen et al. U.S. Patent No. 3,079,745 and in the patents referenced therein. This type of crimp is illustrated in Billion U.S. Patent No. 2,957,224. Edge crimpers of the type disclosed in Pittman et al. U.S. Patent No. 3,047,932 provides suitable crimp. Non-mechanical crimp is suitable, such as the random, three-dimensional nonhelical curvilinear configuration produced with a jet of heated fluid, e.g., as disclosed in Hallden et al. U.S. Patent No. 3,005,251.

The crimped nylon component, which may be referred to as the carrier fiber, of the staple of this invention may be prepared from the same polymer as the uncrimped component, or from a different nylon polymer. Likewise, the crimped fiber may have the same or different denier per filament, the same or different cut length, and the same or different filament cross-section. As pointed out previously, the essential feature is that the uncrimped, high load-bearing staple fiber be mixed with 10 to 50% of a nylon fiber having a crimp index of at least 8% and preferably in the range of from 15% to 30%.

In a preferred embodiment, where it is desired that the two components of the nylon staple of this invention have the same dyeing properties, the crimped portion is prepared in substantially the same manner as the high  $T_7$  uncrimped portion, but with the additional step of crimping being added after the drawing heat-treating step, which may be accomplished either as a separate step or integrated in the drawing heat-treating step. The similar preparation of both components avoids dissimilarities of internal structural features in respects which would cause differences in dye receptivity. The dyeing rates of the two components are nearly equivalent, with a consequent improvement in dyeing uniformity in the finished textile article.

For best results in processing on cotton system equipment, it is preferred that the crimped and uncrimped components of the staple of this invention have substantially the same cut length.

The staple of this invention is readily prepared by combining tows of crimped and uncrimped continuous fibers in the desired proportions and feeding the combined tow to a conventional staple cutter. The product issuing from the cutter is an intimate uniform blend of crimped and uncrimped staple fibers.

In another embodiment, a continuous filament is first crimped and then cut into staple. This crimped fiber is blended with separately cut, uncrimped fiber to serve as the carrier fiber for the uncrimped component.

The birefringence of the yarn is determined according to methods of Heyn, Textile Research Journal 22, No. 513 (1952), and is a measure of structural orientation. The density is measured using density gradient tubes, according to the method of Boyer, Spencer and Wiley, Journal of Polymer Science 1, No. 249 (1946). The density is proportional to the degree of crystallinity of the fiber.

The invention is further illustrated by the following examples which are intended to be illustrative and not limitative.

#### EXAMPLE I

Polyhexamethylene adipamide is melt spun and drawn according to the method described in my U.S. Patent 3,044,250 to give a 2.3 denier per filament (0.256 tex. per filament) uncrimped tow in which the filaments have the following properties: a density of 1.14 grams per cc., a birefringence of 0.0594, a tenacity of 6.6 grams per denier, a break elongation of 22%, a boil-off shrinkage of 5.1%, and a load-bearing capacity at 7% elongation ( $T_7$ ) of 2.3 g.p.d. The crimp index of these filaments is substantially zero. This tow is referred to as the high  $T_7$  component.

Polyhexamethylene adipamide is also used to prepare

two low modulus, commercial grade, crimped tows, A and B, by conventional methods to serve as carrier fibers for the above high  $T_7$  tow. The crimp is that provided by a conventional stuffer box crimpler as disclosed in Hitt U.S. Patent No. 2,311,174. Tow A is composed of filaments having a denier of 1.5 (0.167 tex.), a tenacity of 4.0 g.p.d., a break elongation of 36%, a  $T_7$  value of 0.9 g.p.d., and an average crimp index of 18%. Tow B is composed of filaments having a denier of 3.0 (0.333 tex.), a tenacity of 4.1 g.p.d., a break elongation of 36%, a  $T_7$  value of 0.9 g.p.d., and an average crimp index of 20%.

The uncrimped high  $T_7$  tow is combined with each of tows A and B in weight ratios 20/80, 35/65, and 50/50 (crimped/uncrimped), and cut to staple having a length 1.5 inches. These six staple blends are then picked and carded on cotton system equipment, along with a control item composed of the high  $T_7$  fibers only. The high  $T_7$  control gives excessive card loading as well as poor web cohesion. In contrast, each of the other six staple items 20 exhibits markedly reduced card loading and gives significantly higher web cohesion.

Each of the above seven nylon staple items is used to prepare a nylon/cotton yarn of 50/50 composition by blending the nylon sliver with a middlings cotton sliver 25 on a draw frame. Each of these nylon/cotton blends is split during spinning to produce two yarns, a filling yarn of 17.5/1's cotton count construction, 3.3 twist multiplier, and a warp yarn of 21/1's cotton count, 4.75 twist multiplier. The strength of each product is determined and reported as Lea product (skein break factor) in the table below.

The data in Table I shows that, although substitution of crimped nylon carrier fiber for part of the high  $T_7$  component in the cotton/nylon blend yarn reduces the yarn strength somewhat, the yarn is still stronger than a 100% cotton yarn. This result is in contrast to that obtained with a nylon-cotton blend yarn containing less than 50% nylon in which there is no high  $T_7$  component. Such yarns are always weaker than 100% cotton yarn.

Similar results are obtained when the uncrimped high  $T_7$  component is composed of filaments having a denier of 1.5 (0.167 tex.). Substantially equivalent results are obtained when the nylon fibers of the example are prepared from polycaproamide.

Table I

|    | Spun Yarn Blend Composition |                          |                      |                 | Lea Product  |            |
|----|-----------------------------|--------------------------|----------------------|-----------------|--------------|------------|
|    | Carrier Fiber A, percent    | Carrier Fiber B, percent | High $T_7$ , percent | Cotton, percent | 17.5/1's cc. | 21/1's cc. |
| 50 | -----                       | -----                    | 50                   | 50              | 2,634        | 2,441      |
|    | 10                          | -----                    | 40                   | 50              | 2,386        | 2,135      |
| 55 | 17.5                        | -----                    | 32.5                 | 50              | 2,289        | 2,054      |
|    | 25                          | -----                    | 25                   | 50              | 2,019        | 1,911      |
|    | -----                       | 10                       | 40                   | 50              | 2,332        | 2,085      |
|    | -----                       | 17.5                     | 32.5                 | 50              | 2,260        | 2,002      |
|    | -----                       | 25                       | 25                   | 50              | 1,989        | 1,850      |
| 60 | -----                       | -----                    | -----                | 100             | 1,825        | 1,725      |

#### EXAMPLE II

Web strength is difficult to measure accurately, but is known to be directly proportional to card sliver cohesion. The following experiment is carried out to show the effect of the presence of a carrier fiber on card sliver cohesion, and thereby indicate the effect on web strength.

Selected blends of the high  $T_7$  staple and carrier fibers A and B prepared in Example I are processed through the picker and card to produce card slivers which are tested for strength on a Uster Tester as follows: Card sliver is passed through two sets of two rolls each and between which a speed differential exists such that a small amount (1.78 $\times$ ) of drafting takes place. The downstream roll set is on a flexible mount, and moves back and forth as the sliver cohesion varies. This movement sends an electric signal to a recorder through a transducer cir-

cuit. The recorder is calibrated to read the sliver pull force (i.e., the flexible mount movement) in milligrams.

The strength of each sliver is reported in Table II in terms of milligrams per denier.

Table II

| Spun Yarn Blend Composition |                          |                               | Uster Card Sliver Co-hesion, Mg./Den. |
|-----------------------------|--------------------------|-------------------------------|---------------------------------------|
| Carrier Fiber A, Percent    | Carrier Fiber B, Percent | High T <sub>7</sub> , Percent |                                       |
| 35                          | -----                    | 65                            | 4.7                                   |
| 50                          | -----                    | 50                            | 5.3                                   |
| -----                       | 20                       | 80                            | 5.5                                   |
| -----                       | 35                       | 65                            | 4.7                                   |
| -----                       | 50                       | 50                            | 4.4                                   |
| -----                       | 100                      | (control)                     | 4.0                                   |

The data in the table clearly shows that the blends containing a carrier fiber produce card slivers having a significantly higher strength than the control samples.

## EXAMPLE III

Polyhexamethylene adipamide is melt spun and drawn, according to the method described in my U.S. Patent No. 3,044,250, to become an uncrimped tow identical to the high T<sub>7</sub> sample of Example I.

Polyhexamethylene adipamide is also used to prepare a high modulus crimped tow to serve as carrier fibers for the high T<sub>7</sub> tow of this Example III. This crimped tow may be prepared either by crimping high T<sub>7</sub> tow in the integrated process of drawing and crimping, or by a separate step. In either case, a stuffer box crimper is used, as disclosed in Hitt U.S. Patent No. 2,311,174, and sufficient plasticity of the tow may be achieved through moisture addition to facilitate crimp formation. This crimped tow is composed of filaments having a denier of 3.0, a tenacity of 4.1 g.p.d., a break elongation of 36%, a T<sub>7</sub> value of 0.9 g.p.d., and an average crimp index of 8%.

A staple blend of the uncrimped high T<sub>7</sub> tow for this Example III (84%), with the high modulus crimped tow of this Example III (16%), is picked and carded on cotton system equipment and a significantly high web cohesion as well as a reduced card loading is experienced.

A nylon/cotton yarn of 18/82 composition is prepared by blending the nylon blend sliver of this Example III with a middlings cotton sliver on a draw frame. This nylon/cotton blend is split during spinning to produce two yarns, a filling yarn of 17.5/1's cotton count construction, 3.3 twist multiplier, and a warp yarn of 21/1's cotton count, 4.75 twist multiplier. The Lea products of the warp yarn and of the filling yarn show that each yarn is much stronger than an equivalent 100% cotton yarn. Web strength for the nylon staple blend of this Example III is significantly higher than the strength of an all-high T<sub>7</sub> control.

The warp yarn and the filling yarn of this example are woven into denim and other heavy service fabrics which unexpectedly exhibit superior serviceability.

The improvement afforded by the nylon staple blends of this invention is obtained over a wide range of filament deniers, e.g., from 1.2 to 15 denier and above. Likewise, the invention is not limited to any particular length. Any staple length suitable for blending with cotton may be used, e.g., 1", 1 1/8", 1 1/2", 1 3/4", 2", 2 1/2", 3", 4", and others. Where the nylon blend is to be used for reinforcing fibers other than cotton (such as viscose rayon, acetate rayon, and other cellulosic derivatives, as well as protein fibers and such synthetic fibers as polyacrylonitriles and polyolefins) other staple cut lengths may be used as suitable for each fiber to be reinforced.

Although the invention has been illustrated in the ex-

amples primarily with nylon staple fibers prepared from polyhexamethylene adipamide, other synthetic linear condensation polymer fibers, including both nylon and polyester fibers, may be used. The invention may be applied generally to fibers of any synthetic linear polymer having recurring units of the formula



- 10 as integral parts of the main polymer chain, wherein R is hydrogen or a monovalent hydrocarbon radical, the average number of carbon atoms separating the amide groups being at least two, said polycarbonamide having an intrinsic viscosity of at least about 0.4, as defined in Carrothers U.S. Patent No. 2,130,948, dated September 20, 1938. Particular polycarbonamides included among those which are useful in this invention are as follows: polyhexamethylene adipamide, polyhexamethylene sebacamide, polymerized 6-aminocaproic acid, polytetramethylene sebacamide, polytetramethylene adipamide, polymetaxylylene adipamide, the polyamide from bis(4-aminocyclohexyl)methane and azelaic acid, sebacic acid or decamethylene-1,10-dicarboxylic acid, and the polyamide from 2-methylhexamethylene diamine and terephthalic acid.
  - 15 The invention is also applicable to various copolymers, either block or random, such as the copolymer of polyhexamethylene adipamide and polyhexamethylene isophthalamide, and the copolymer of polyhexamethylene adipamide and polyhexamethylene-t-butyl isophthalamide.
  - 20
  - 25
  - 30
  - 35
  - 40
- The nylon staples of this invention may contain conventional delustrants, dye modifiers, antistatic agents, antioxidants, heat stabilizers and the like. Suitable staple finishes may be added to the fibers as desired.

The present invention offers a distinct improvement over the prior art. It provides for improved and more economical processing of nylon staples especially suitable for reinforcing natural fibers such as cotton. The blended yarn produced may be fashioned into wearing apparel, industrial fabrics, sheeting, and like articles which are characterized by improved wear and abrasion resistance.

Since many different embodiments of the invention may be made without departing from the spirit and scope thereof, it is to be understood that the invention is not limited by the specific illustrations except to the extent defined in the following claims.

I claim:

1. A combination of crimped and uncrimped nylon staple fiber suitable for blending with cotton fiber, comprising a mixture of 50% to 90% of uncrimped nylon staple fiber characterized by a load-bearing capacity of at least 2.1 grams per denier at 7% elongation and a boil-off shrinkage of not over 6%, both properties measured after 9 days' slack ageing, and 50% to 10% of crimped nylon staple fibers having a crimp index of at least 8%.
2. A product as defined in claim 1 wherein the nylon fibers are of polyhexamethylene adipamide.
3. A product as defined in claim 2 wherein the uncrimped fibers are further characterized by a birefringence of at least 0.0590 and an average density above about 1.139 grams per cubic centimeter.
4. A product as defined in claim 1 wherein the crimped stable fiber has a crimp index of 15% to 30%.
5. A product as defined in claim 1 wherein the crimped staple fiber component is obtained by crimping said uncrimped staple fiber.
6. A yarn composed of a blend of cotton and a mixture of 50% to 90% of uncrimped nylon staple fiber characterized by a load-bearing capacity of at least 2.1 grams per denier at 7% elongation and a boil-off shrinkage of not over 6%, both properties measured after 9 days slack ageing, and 50% to 10% of crimped nylon staple fiber having a crimp index of at least 8%.
7. A product as defined in claim 1 wherein the uncrimped fibers are further characterized by a birefringence of at least 0.0590 and an average density above about 1.139 grams per cubic centimeter.
8. A product as defined in claim 1 wherein the crimped stable fiber has a crimp index of 15% to 30%.
9. A product as defined in claim 1 wherein the crimped staple fiber component is obtained by crimping said uncrimped staple fiber.
10. A product as defined in claim 1 wherein the uncrimped fibers are further characterized by a birefringence of at least 0.0590 and an average density above about 1.139 grams per cubic centimeter.
11. A product as defined in claim 1 wherein the crimped stable fiber has a crimp index of 15% to 30%.
12. A product as defined in claim 1 wherein the crimped staple fiber component is obtained by crimping said uncrimped staple fiber.
13. A product as defined in claim 1 wherein the uncrimped fibers are further characterized by a birefringence of at least 0.0590 and an average density above about 1.139 grams per cubic centimeter.
14. A product as defined in claim 1 wherein the crimped stable fiber has a crimp index of 15% to 30%.
15. A product as defined in claim 1 wherein the crimped staple fiber component is obtained by crimping said uncrimped staple fiber.
16. A product as defined in claim 1 wherein the uncrimped fibers are further characterized by a birefringence of at least 0.0590 and an average density above about 1.139 grams per cubic centimeter.
17. A product as defined in claim 1 wherein the crimped stable fiber has a crimp index of 15% to 30%.
18. A product as defined in claim 1 wherein the crimped staple fiber component is obtained by crimping said uncrimped staple fiber.
19. A product as defined in claim 1 wherein the uncrimped fibers are further characterized by a birefringence of at least 0.0590 and an average density above about 1.139 grams per cubic centimeter.
20. A product as defined in claim 1 wherein the crimped stable fiber has a crimp index of 15% to 30%.
21. A product as defined in claim 1 wherein the crimped staple fiber component is obtained by crimping said uncrimped staple fiber.
22. A product as defined in claim 1 wherein the uncrimped fibers are further characterized by a birefringence of at least 0.0590 and an average density above about 1.139 grams per cubic centimeter.
23. A product as defined in claim 1 wherein the crimped stable fiber has a crimp index of 15% to 30%.
24. A product as defined in claim 1 wherein the crimped staple fiber component is obtained by crimping said uncrimped staple fiber.
25. A product as defined in claim 1 wherein the uncrimped fibers are further characterized by a birefringence of at least 0.0590 and an average density above about 1.139 grams per cubic centimeter.
26. A product as defined in claim 1 wherein the crimped stable fiber has a crimp index of 15% to 30%.
27. A product as defined in claim 1 wherein the crimped staple fiber component is obtained by crimping said uncrimped staple fiber.
28. A product as defined in claim 1 wherein the uncrimped fibers are further characterized by a birefringence of at least 0.0590 and an average density above about 1.139 grams per cubic centimeter.
29. A product as defined in claim 1 wherein the crimped stable fiber has a crimp index of 15% to 30%.
30. A product as defined in claim 1 wherein the crimped staple fiber component is obtained by crimping said uncrimped staple fiber.
31. A product as defined in claim 1 wherein the uncrimped fibers are further characterized by a birefringence of at least 0.0590 and an average density above about 1.139 grams per cubic centimeter.
32. A product as defined in claim 1 wherein the crimped stable fiber has a crimp index of 15% to 30%.
33. A product as defined in claim 1 wherein the crimped staple fiber component is obtained by crimping said uncrimped staple fiber.
34. A product as defined in claim 1 wherein the uncrimped fibers are further characterized by a birefringence of at least 0.0590 and an average density above about 1.139 grams per cubic centimeter.
35. A product as defined in claim 1 wherein the crimped stable fiber has a crimp index of 15% to 30%.
36. A product as defined in claim 1 wherein the crimped staple fiber component is obtained by crimping said uncrimped staple fiber.
37. A product as defined in claim 1 wherein the uncrimped fibers are further characterized by a birefringence of at least 0.0590 and an average density above about 1.139 grams per cubic centimeter.
38. A product as defined in claim 1 wherein the crimped stable fiber has a crimp index of 15% to 30%.
39. A product as defined in claim 1 wherein the crimped staple fiber component is obtained by crimping said uncrimped staple fiber.
40. A product as defined in claim 1 wherein the uncrimped fibers are further characterized by a birefringence of at least 0.0590 and an average density above about 1.139 grams per cubic centimeter.
41. A product as defined in claim 1 wherein the crimped stable fiber has a crimp index of 15% to 30%.
42. A product as defined in claim 1 wherein the crimped staple fiber component is obtained by crimping said uncrimped staple fiber.
43. A product as defined in claim 1 wherein the uncrimped fibers are further characterized by a birefringence of at least 0.0590 and an average density above about 1.139 grams per cubic centimeter.
44. A product as defined in claim 1 wherein the crimped stable fiber has a crimp index of 15% to 30%.
45. A product as defined in claim 1 wherein the crimped staple fiber component is obtained by crimping said uncrimped staple fiber.
46. A product as defined in claim 1 wherein the uncrimped fibers are further characterized by a birefringence of at least 0.0590 and an average density above about 1.139 grams per cubic centimeter.
47. A product as defined in claim 1 wherein the crimped stable fiber has a crimp index of 15% to 30%.
48. A product as defined in claim 1 wherein the crimped staple fiber component is obtained by crimping said uncrimped staple fiber.
49. A product as defined in claim 1 wherein the uncrimped fibers are further characterized by a birefringence of at least 0.0590 and an average density above about 1.139 grams per cubic centimeter.
50. A product as defined in claim 1 wherein the crimped stable fiber has a crimp index of 15% to 30%.
51. A product as defined in claim 1 wherein the crimped staple fiber component is obtained by crimping said uncrimped staple fiber.
52. A product as defined in claim 1 wherein the uncrimped fibers are further characterized by a birefringence of at least 0.0590 and an average density above about 1.139 grams per cubic centimeter.
53. A product as defined in claim 1 wherein the crimped stable fiber has a crimp index of 15% to 30%.
54. A product as defined in claim 1 wherein the crimped staple fiber component is obtained by crimping said uncrimped staple fiber.
55. A product as defined in claim 1 wherein the uncrimped fibers are further characterized by a birefringence of at least 0.0590 and an average density above about 1.139 grams per cubic centimeter.
56. A product as defined in claim 1 wherein the crimped stable fiber has a crimp index of 15% to 30%.
57. A product as defined in claim 1 wherein the crimped staple fiber component is obtained by crimping said uncrimped staple fiber.
58. A product as defined in claim 1 wherein the uncrimped fibers are further characterized by a birefringence of at least 0.0590 and an average density above about 1.139 grams per cubic centimeter.
59. A product as defined in claim 1 wherein the crimped stable fiber has a crimp index of 15% to 30%.
60. A product as defined in claim 1 wherein the crimped staple fiber component is obtained by crimping said uncrimped staple fiber.
61. A product as defined in claim 1 wherein the uncrimped fibers are further characterized by a birefringence of at least 0.0590 and an average density above about 1.139 grams per cubic centimeter.
62. A product as defined in claim 1 wherein the crimped stable fiber has a crimp index of 15% to 30%.
63. A product as defined in claim 1 wherein the crimped staple fiber component is obtained by crimping said uncrimped staple fiber.
64. A product as defined in claim 1 wherein the uncrimped fibers are further characterized by a birefringence of at least 0.0590 and an average density above about 1.139 grams per cubic centimeter.
65. A product as defined in claim 1 wherein the crimped stable fiber has a crimp index of 15% to 30%.
66. A product as defined in claim 1 wherein the crimped staple fiber component is obtained by crimping said uncrimped staple fiber.
67. A product as defined in claim 1 wherein the uncrimped fibers are further characterized by a birefringence of at least 0.0590 and an average density above about 1.139 grams per cubic centimeter.
68. A product as defined in claim 1 wherein the crimped stable fiber has a crimp index of 15% to 30%.
69. A product as defined in claim 1 wherein the crimped staple fiber component is obtained by crimping said uncrimped staple fiber.
70. A product as defined in claim 1 wherein the uncrimped fibers are further characterized by a birefringence of at least 0.0590 and an average density above about 1.139 grams per cubic centimeter.
71. A product as defined in claim 1 wherein the crimped stable fiber has a crimp index of 15% to 30%.
72. A product as defined in claim 1 wherein the crimped staple fiber component is obtained by crimping said uncrimped staple fiber.
73. A product as defined in claim 1 wherein the uncrimped fibers are further characterized by a birefringence of at least 0.0590 and an average density above about 1.139 grams per cubic centimeter.
74. A product as defined in claim 1 wherein the crimped stable fiber has a crimp index of 15% to 30%.
75. A product as defined in claim 1 wherein the crimped staple fiber component is obtained by crimping said uncrimped staple fiber.

7. A yarn as defined in claim 6 wherein the nylon fibers are of polyhexamethylene adipamide.

8. A yarn as defined in claim 6 wherein the crimped staple fiber has a crimp index of 15% to 30%.

9. A yarn as defined in claim 6 composed of about 50% to 82% of cotton, the remainder being the mixture of crimped and uncrimped nylon staple fiber, the yarn having a Lea products strength greater than that of an equivalent 100% cotton yarn.

References Cited by the Examiner

UNITED STATES PATENTS

|           |       |                |          |
|-----------|-------|----------------|----------|
| 1,172,439 | 9/39  | Dreyfus et al. | 57—140   |
| 2,636,222 | 4/53  | Wilkie         | 19—145.5 |
| 2,851,737 | 9/58  | Hunter et al.  | 19—145.5 |
| 3,007,227 | 11/61 | Moler          | 57—140   |

MERVIN STEIN, Primary Examiner.